

J. D. HATHAWAY,

METHOD AND APPARATUS FOR COATING METALLIC ARTICLES.  
APPLICATION FILED SEPT. 20, 1916.

1,248,107.

Patented Nov. 27, 1917.



Inventor  
Joseph D. Hathaway:  
by J. S. Roberts  
Atty's.

# UNITED STATES PATENT OFFICE.

JOSEPH D. HATHAWAY, OF MONTREAL, QUEBEC, CANADA, ASSIGNEE, BY MESNE ASSIGNMENTS, TO WESTERN ELECTRIC COMPANY, INCORPORATED, OF NEW YORK, N. Y., A CORPORATION OF NEW YORK.

## METHOD AND APPARATUS FOR COATING METALLIC ARTICLES.

1,248,107.

Specification of Letters Patent. Patented Nov. 27, 1917.

Application filed September 20, 1916. Serial No. 121,157.

To all whom it may concern:

Be it known that I, JOSEPH D. HATHAWAY, a citizen of the United States, residing at Montreal, in the Province of Quebec, Canada, have invented certain new and useful Improvements in the Methods and Apparatus for Coating Metallic Articles, of which the following is a full, clear, concise, and exact description.

10 This invention relates to an improved method and apparatus for coating metallic articles, and more particularly to an improved and efficient method and apparatus for applying to metallic articles a very thin and uniform coating of another metal. More specifically the invention relates to an improved method and apparatus for applying a very thin coating of tin to copper wire and then subjecting the coated conductor to 20 a coating of insulating enamel.

One of the objects of this invention is to produce a method and apparatus for covering articles with a coating of another metal in which the metallic coating is so finely distributed that the coating will have no tendency to run when subjected to a coating of baked enamel at a temperature as high, or higher than the melting temperature of the coating metal.

25 Another object of the invention is to produce an improved method and apparatus for procuring coated wires of the exact size or gage desired, by utilizing an uncoated wire which is slightly over size, subjecting it to a coating of another metal and then drawing the coated wire to the exact size desired.

30 A further object of this invention is the production of an improved method and apparatus for materially increasing the speed at which metallic coatings are applied to wires and to apply a coating which is exceeding thin and which is evenly distributed.

Another object is the production of a 35 method and apparatus for applying to copper conductors a very thin, smooth and evenly distributed coating of tin and then applying to said tinned wire a smooth and even coating of baked insulating enamel.

Other features of this invention will become apparent from the following description and the appended claims.

This invention is useful and applicable whenever it is desired to apply to an article a very thin and evenly distributed me-

tallic coating. In the preferred embodiment 55 of the invention herein described it has been applied to the covering of copper wires with a coating of tin, but the invention is not limited to the specific embodiment described which is susceptible to many variations and 60 applications without departing from its spirit and scope as set forth in the appended claims.

The practice of tinning metal surfaces which are to be soldered is old and well 65 known. Likewise it is an old and universal practice to tin wires, which are used in the construction of electric apparatus, before the wires are given a coating of insulation. Consequently ever since the practicability of the 70 baked enamel wire was established attempts have been made to develop a suitable and an efficient apparatus and method for producing tinned wire over which a smooth and evenly distributed surface of baked enamel 75 could be applied. The development of this process was extremely difficult because the melting temperature of the coating metal tin, was somewhat lower than the temperature required in the process of coating the 80 wire with the baked enamel. Therefore, when attempts were made to subject a tinned wire to a coating of baked enamel, the tinned coating on the surface of the wire would run into globules and form small horny 85 projections of tin on the surface of the enameled wire. These horny projections in the process of coating the wire with enamel would be covered with enamel, but in the subsequent handling of the wire the enamel 90 on these projections would chip and break off and thus expose bare, uninsulated surfaces on the wire. As these uninsulated surfaces would develop in the handling and the working of the wire, the use of tinned 95 enamel wire was rather unsatisfactory, as these bared spots in the wire would frequently not manifest themselves until the wire had been used in the manufacture of apparatus.

100 It was, therefore, very desirable to devise a method and apparatus whereby a very thin coating of tin could be applied to wire which would have no tendency to run when subjected to the temperature required for 105 coating the tinned wire with a baked enamel. The herein described method and apparatus produces a tinned, baked enamel wire, which

has a smooth even surface and on which the tin and enamel coatings are very evenly distributed and on which there are no bare or uninsulated spots.

5 The apparatus used in the application of the process is illustrated in the accompanying drawings, in which—

Figure 1 is a side elevation and

Fig. 2 is a plan view of the complete machine; and

Fig. 3 illustrates a vertical section of the die housing showing the relative position of the die in the metallic bath.

As illustrated in Figs. 1 and 2, the complete machine is composed of four units—a combined acid bath and spool holder 1, a tin bath 2, a water bath 3 and a wire take-up mechanism 4. The acid bath as shown at 1 consists of a container 7 for holding the acid, in the bottom of which is placed a felt pad. On the right-hand side of the container are mounted a series of guiding posts 8 for guiding the wire under the roller 9 into the acid container 7. Extending upwardly to the right from the frame holding the acid container is an arm 12, on which are mounted a plurality of spindles 14. These spindles serve to receive the feeding spools 15 on which is wound the wire which is to be coated. In the preferred embodiment of the apparatus here illustrated provisions are made for mounting six spools, but it will be evident that the apparatus can be readily designed for the mounting of any desired number of spools. Removably mounted in the acid bath container are a plurality of lead weights 16 equal in number to the number of spools mounted on the upright member 12. The lower surface of these lead weights is covered with a piece of felt, and the lead weight in conjunction with this piece of felt serves to hold the wire fed through the acid container in the acid between the felt pad mounted in the bottom of the container and the felt on the bottom of the lead weight 16. To the left of the acid container is mounted an acid removing means 18. Any suitable means can be employed for this purpose, but in the device here illustrated a rubber wiper is used. A guide roller 20 is placed to the left of the rubber wiper 18 over which the wire passes after leaving the rubber wiper.

The tin bath unit 2 comprises a housing 21 mounted on suitable standards and in which is placed a container 22 which holds the fluid tin. To the right of the tin bath container 22 is mounted a roller 23, which serves to guide the wire on its way into the bath. Supported on the housing 21 is an adjustable arm 25 which carries a roller 26 and a die holder 27. This adjustable arm 25 is capable of movement in a vertical direction on the post 30. This movement of the adjustable arm 25 is provided for conven-

ience in stringing the wire through the tin bath. Thus when the arm 25 is moved to its extreme upward position, the die holder 27 and the roller 26 are removed from the tin bath, and the wire can be conveniently strung under the roller and through the die clamped in the holder 27. The tin in the container 22 may be heated and maintained in a molten condition by any well-known means. In the preferred embodiment of the invention here illustrated the heating of the container 22 is accomplished by a gas flame, the gas being supplied through the feed pipe 31. To the right of the die and supported on the housing 21 are another series of guiding posts 32 and the guide rollers 33 and 34.

The water unit 3 consists of a water container 36, in which is mounted a guide roller 37 which serves to hold the wire immersed in the water as it passes through the water unit 3. Supported on the left face of the water unit 3 is a water removing means 39. This water removing means serves to dry the wire after it leaves the water bath, and any suitable means may be employed for this purpose. A rubber wiper such as shown as 39 has proved very satisfactory. The water in the water container 36 is constantly circulated so as to cool the wire and also to more readily remove any trace of acid which may be left on the wire.

The wire take-up unit 4 is composed of suitable standards on which are supported a series of capstans, such as 41, around which the wire is fed and from where the wire is led to a suitable take-up spool, such as 42, on which the finished wire is wound. The capstans on the take-up mechanism 4 are belt driven by any suitable source of power, such as 44, and the driving mechanism is so arranged that each capstan may be separately operated. Mounted between the capstan 41 and the take-up spool 42 is a distributor 45 which serves to uniformly distribute the wire over the surface of the spool. The take-up spool 42 is frictionally driven, thereby providing a tension which is practically uniform for winding the wire on the spools 42. The capstans 41 and the spools 42 are driven from the source of power 44 by any suitable means of belt or chain drive.

A plurality of rollers 47, one for each wire, are attached to the right face of the water unit 3. Each roller 47 is mounted on a bell crank 48 pivoted at 49. The lower end of each bell crank 49 is connected by any suitable means to a lever 52 which is pivoted at 53. Secured to the lever 52 is a spring 54 which serves as a brake for the spool 42. Thus, if one of the strands of wire should break, the bell crank associated with said wire, due to its weight, will drop by gravity, and by means of the connecting link 56, the lever 52 will be moved about its pivot 53, 130

and will apply the brake spring 54 to the feed spool 14. Consequently whenever a break occurs in a strand of wire, a brake will be applied to the associated feed spool 5 and thus prevent further unrolling of the wire and the tangle which would result from the continued feeding of wire after a strand had been broken.

Fig. 3 illustrates a vertical section of the 10 die and the relative position of the die in the tin bath. The die 60 is mounted in a steel ring 61, which in turn is mounted in a cast-iron housing 59. This housing is clamped into the die holder 27 unitary with the lower 15 part of the downwardly extending arm 25, by a set screw 62. The die proper 60 is placed in the fluid tin so that it always remains submerged during the process of tinning the wire and in which process it acts 20 to wipe the surplus tin from the wire as the wire leaves the tin bath. This die may be constructed of any exceedingly hard material which can stand the severe use to which it is put. In the preferred form of this invention a diamond die has been used and its 25 use has been very satisfactory, but this invention is not limited to the use of a diamond die, as any other stones, and possibly some metals, would be hard enough to stand 30 the severe use to which the die is subjected.

The process of coating wire by means of the apparatus which has been described in detail in the foregoing will now be considered. In this process of tinning copper 35 wire, the wire is first strung through the four units of the machine and the machine is then set into operation. Since each strand of wire is strung through the machine in the same manner, the description of this operation 40 will be confined to one strand of wire. A spool containing copper wire to be tinned is placed on the spindle 14 and the wire is threaded through the guiding posts 8, under the roller 9 and through the acid container 45 between the felt pads to the acid remover 18. From there the wire is fed over the rollers 20 and 23, under the roller 26, through the diamond die 60 and thence through the guiding posts 32, and over the rollers 33 and 50 34. In stringing this wire under the roller 26 and through the diamond die 60, the arm 25 is retained in its topmost position, in which position the roller 26 and the die 60 are not in contact with the molten tin. 55 From the roller 34 the wire is fed under the roller 27 and roller 37 and thence through the water drying means 39, the capstans 41, about which two or three turns are taken, and then through the distributor 45 and on 60 to the take-up spool 42.

When the six strands of wire have been thus threaded through the machine, the six arms 25 are lowered so that the dies 60 will be immersed in the tin solution, as shown in 65 Fig. 3, it being understood, of course, that

the tin in the container 22 has been brought to a fluid state by means of a gas flame directed to the bottom of the container 22. After the dies have been lowered into the fluid tin, power is applied by means of the 70 driving means 44, which, through suitable transmitting means, will turn the various capstans 41 and the take-up spools 42, and thus cause the drawing of the wire from the delivery spools 14 through the units 1, 2, 3 75 and 4, as described above. The wire in passing through the tin in the container is thoroughly covered with tin, and in its passage through the die 60 the surplus tin is removed from the wire, leaving a very 80 thin, uniformly distributed coating of tin on the copper wire. This coating on the copper wire is so thin that it approximates only about three milligrams per square inch. The die 60 contained in the tinning bath 85 is bored to the size of the wire which is ultimately desired and consequently if the wire which is being tinned is the exact size of the ultimately desired coated or tinned wire, then the coated wire in leaving the tin bath 90 will be subjected to a very slight drawing operation, in addition to the wiping operation, because of the thin film of tin with which the wire is coated. In the operation of this process it has been found desirable 95 to use an uncoated copper wire which is slightly over size—that is a wire whose gage is just slightly greater than the gage of the desired coated wire. When an over sized wire of this kind is used, it is obvious that 100 the drawing operation in the die 60 is somewhat greater than when an uncoated wire of the gage of the ultimate coated wire is used. The use of an oversized wire is not essential, and satisfactory results can be obtained with wire drawn to a gage equal to 105 the gage of the ultimately desired coated wire.

In this process of coating copper wire with tin, each strand of wire is drawn through 110 the tin at a rate of about 500 feet per minute and the operation is continuous until all the bare copper wire is removed from the supply spool 14 and the tinned copper wire is wound on the take-up spool 42.

When the wire has thus been tinned and wound on the spool 42, the spool 42 is removed from the take-up mechanism and placed on the supply spindle of a machine designed for coating wires with insulating 120 enamel. A machine for this purpose is disclosed and described in U. S. Patent to G. Gustave, No. 1,004,251. The tinned copper wire wound on spool 42 of the unit 4 of Fig. 1 is then given the treatment disclosed 125 in said patent. In this process of coating wire with baked enamel, the wire is subjected to a temperature which is equal to or slightly higher than the melting point of tin. For this reason when it is attempted 130

to coat wire tinned in the ordinary manner with a coating of baked enamel, the tin has a tendency to run and form in globules on the wire. These globules in the coating process result in thorny projections on the surface of the wire from which the enamel coating will readily chip and thereby surfaces of bare wire are exposed. Further, this tendency of the tin to run results in a very uneven, rough coating of enamel. However, when wire as tinned by the process as above described, is subjected to an enamel baking process of the kind described in the aforesaid patent, the tin has no tendency to run, and the resulting enameled wire is delivered from the baking furnace with an even, smooth surface of baked enamel over the coating of tin, which latter coating is not disturbed in the least by the baking process.

In the description of the apparatus for applying this improved process a preferred embodiment has been described, but obviously this invention is not limited to that specific embodiment, but is capable of many variations and applications without departing from its spirit and scope as outlined in the following claims.

What is claimed is:

- 30 1. The process of coating wires with a coating of another metal which consists in subjecting the wire to a bath of the coating metal and then drawing the coated wire through a die of a smaller gage than that of the uncoated wire.
- 25 2. The process of covering copper wires with a coating of tin which consists in subjecting the wire to a molten tin bath and then drawing the coated tinned wire through a wiping die of the gage of the uncoated wire to exert a drawing effect upon the coated wire and, thereby applying to the copper wire an exceedingly thin coat of tin.
- 40 3. The process of coating wires with a coating of another metal which consists in subjecting the wire to a bath of the coating metal and then drawing the coated wire through a die which is maintained submerged in the bath of the coating metal.
- 45 4. The process of covering copper wires with a coating of tin which consists in subjecting the copper wire to a molten tin bath and then drawing the coated tinned wire through a wiping die which is maintained submerged in the tin bath.
- 50 5. The method of producing wires covered with a coating of another metal of a desired size or gage which consists in subjecting an over size uncoated wire to a bath of the coating metal and then drawing the coated conductor through a die of the desired size.
- 55 6. The method of producing tinned copper wire of a desired size or gage which consists in subjecting an over size copper wire

to a bath of tin and then drawing the tinned copper wire through a die of the desired size.

7. The process of covering wires with a very thin, fine, evenly distributed coating of metal and insulating enamel, which consists in subjecting the wire to a bath of the coating metal, then drawing the coated wire through a die of a smaller gage than the uncoated wire and finally subjecting the metal so coated to a bath of insulating enamel.

8. The process of covering copper wires with a fine coating of tin which consists in passing the copper wire through an acid bath, removing the acid from the wire, then subjecting the wire to a bath of fluid tin and finally drawing the tinned wire through a die of a size slightly smaller than the size of the original copper wire.

9. The process of covering copper wires with a very thin primary coating of tin and a secondary coating of insulating enamel, which consists in treating the copper to a bath of fluid tin, then drawing the tinned copper wire through a die to a size smaller than the original copper wire and finally subjecting the tinned wire to a bath of the insulating enamel.

10. The process of covering copper wire with a very thin, primary coating of tin and secondary coating of insulating enamel, which consists in treating the copper wire to a bath of molten tin, then drawing the tinned copper wire through a die to a size smaller than the original copper wire and finally subjecting the tinned wire to a bath of the insulating enamel at a temperature equal to, or higher than the melting point of tin.

11. The method of providing a metal article with an exceedingly thin coating of another metal, which consists in passing the article to be coated through a bath of the coating metal and then drawing the coated article through a die to produce the desired size.

12. The process of producing a tinned copper wire having an outside coating of insulating enamel, which consists in subjecting the copper wire to a fluid bath of tin and then drawing the coated wire through a die to reduce the tinned coating to a degree of thinness which will prevent the running of the tin coating when the coated wire is treated with a coating of insulating enamel at a temperature exceeding that of the melting point of tin.

13. In a machine for coating wire with another metal the combination with a wire feeding mechanism, of an acid bath and acid removing device for cleaning the wire, a metal bath for coating the wire, a die for drawing the coated wire to the desired size, a water bath, a water removing means and a wire take-up mechanism.

14. In a machine for coating wire, the combination with a wire feeding means, of a metal coating means and a die for drawing the coated wire to the desired size.
- 5 15. In a machine for coating copper wire, the combination with a wire feeding means, of an acid bath and acid removing means for cleaning the wire, a tin bath for coating the wire, a die for drawing the tinned copper
- 10 wire to the desired size, a water bath, a water removing means and a wire take-up mechanism for receiving the finished wire.
- 15 16. In a machine for coating wire, a wire feeding means, a wire guiding means whereby the wire is guided through, an acid bath, an acid removing means, a metal bath for coating the wire, a die for drawing the coated wire to the desired size, a water bath, a water removing means and a wire take-up
- 20 means for receiving the finished wire.
17. In a machine for tinning copper wire, a combination with a wire feeding means and a wire guiding means whereby the copper wire is guided through, an acid bath,
- an acid removing means, a tin bath for tinning the wire, a die for drawing the tinned copper wire to the desired size, a water bath, a water removing means and a wire take-up means for receiving the coated wire.
18. In a machine for simultaneously tinning a plurality of copper wires, the combination with wire feeding means, of means for guiding said wires, a tinning bath for said wires, a plurality of dies one for each wire for drawing the tinned copper wire to the size desired, and a wire take-up mechanism comprising means for uniformly drawing the wires from the feeding means through the guiding means and the tinning bath.
- 30 35 40

In witness whereof, I hereunto subscribe my name this twenty eight day of July A. D., 1916.

JOSEPH D. HATHAWAY.

Witnesses:

L. A. MORELAND,  
H. D. KEMP.